

# UNITED STATES PATENT OFFICE.

WILLIAM BOWMAN BALLANTINE, OF LONDON, ENGLAND, ASSIGNOR TO THE EMPIRE (ALLOY) STEEL CORPORATION, LIMITED, OF LONDON, ENGLAND, A BRITISH CORPORATION.

## PRODUCTION OF METALLIC ALLOYS.

1,386,981.

Specification of Letters Patent.

Patented Aug. 9, 1921.

No Drawing.

Application filed August 19, 1920. Serial No. 404,550.

To all whom it may concern:

Be it known that I, WILLIAM BOWMAN BALLANTINE, a subject of the King of England, residing in London, England, have 5 invented certain new and useful Improvements in the Production of Metallic Alloys, of which the following is a specification.

This invention consists in improvements in or relating to the production of metallic 10 alloys, particularly ferro-alloys, such for example as ferro-chrome, and the object is to render the production more economical.

Various economical methods are known 15 for the production of ferro-alloys containing a higher percentage of carbon, such as 1% to 8% of carbon. These ferro-alloys with a higher percentage of carbon are manufactured, for example, in blast furnaces, electric furnaces, and in other ways, at a 20 cost which enables them to be sold at a price very much below that of ferro-alloys with a low carbon content. The object of this invention is to provide means for the economical production of ferro-alloys having 25 a low percentage of carbon (say 0.15% or less of carbon).

According to this invention the process for the economical production of ferro-alloys containing a low percentage of carbon 30 consists in taking a high-carbon ferro-alloy, remelting the same, if necessary, for example in a cupola furnace, running the molten metal directly into a converter of the blast—or Bessemer—type, and blowing 35 atmospheric air through the molten mass until the proportion of carbon has been reduced to any desired percentage, after which the alloy is used or treated in any usual way.

40 Where the ferro-alloy dealt with in this manner requires, for its fusion, a temperature higher than that obtainable in the ordinary coke-fired cupola furnace, the air supplied to the cupola furnace or to the 45 Bessemer or like converter, or to both, may be pre-heated either by utilizing the waste heat of the said cupola furnace or the converter, or in any other suitable manner.

According to one feature of this invention, the process for the production of ferro-chrome alloys of low carbon content comprises submitting crude ferro-chrome, obtained, for example, by reduction of chromite in an electrical furnace, to decarburiza-

tion in a Bessemer or like converter. Preferably, the crude ferro-chrome is mixed with a molten mild basic steel prior to treatment in the converter. According to this invention also the molten alloy produced in the converter may be treated, either before or after tapping, with a thermo-reduction mixture containing a pure chromium compound, in order to compensate for loss during the process or to provide the desired percentage of chromium in the final alloy. In the preferred method of operation, the thermo-reduction mixture is added to the molten alloy in compacted form, for example, in a canister or as a briquet. Oxids of chromium and iron, either alone or in combination, may be used to assist the oxidation of the excess of carbon in the converter.

The crude ferro-chrome may be prepared by the reduction of chromite in an electric furnace, the charge consisting of chromite and anthracite coal, or coke, in the calculated respective proportions. Steel scrap or like material may form part of the charge, as desired. Any of the usual types of furnace may be employed, such as the Heroult, or Girod, or other type of furnace employed for the production of electric steels. The ferro-chrome obtained is usually fairly rich in carbon, although it is possible under certain conditions, for example, by prolonged heating of the impure alloy in an arc furnace with special slags as chromite, lime and fluor-spar, to produce an alloy containing less than 2 per cent. of carbon. The further decarburization is effected in the Bessemer converter as in the manner for the treatment of molten pig iron, the progress of the oxidation being judged, as in the usual Bessemer operation, by the flame colors and other phenomena familiar to those skilled in the art.

The converter may be a baby converter capable of holding a charge of about 5 tons, and it may be lined with an acidic or a basic lining, or a neutral refractory, such as chromite, may be used. As stated, oxids of chromium and iron may be employed to assist the oxidation process.

By treatment in the converter, the carbon content of the ferro-chrome may be reduced to about 1 per cent., or the oxidation may be continued until a very low carbon content is obtained. As the operation proceeds more

of the alloying metals are oxidized and pass into the slag, but slags rich in oxide of chromium may be used as part of the charge in the electric furnace in the process for the 5 production of the crude ferro-chrome.

The admixture of the crude ferro-chrome with mild basic steel, prepared, for example, in the same or in an adjacent converter, facilitates the preparation of the ferro-chrome 10 charge and the subsequent decarburization.

By a thermo-reduction mixture is meant any metal, element or compound or a mixture of these in any proportion which has or have the property of reducing the oxides, 15 haloid or other compounds of the combined metal or metals to form the free metal or metals, the process of reduction being accompanied by the evolution of heat. Aluminium in the powdered or granulated form 20 is perhaps the best known of the reducing agents, in this reaction, but other well-known reagents are calcium silicid, calcium, magnesium, calcium carbide, silicon, and so on, and these and other such suitable 25 reagents may be used either separately or in any combination. The chromium in the thermo-reduction mixture may be in the form of chromite, or of a pure compound of chromium, such as chromium oxid, or of a 30 mixture of these, in association with one or more of the known thermo-reducing agents such as those mentioned. The amount of such a mixture added is such as to enrich the molten alloy by the amount of metallic 35 chromium necessary to give the final ferro-chrome alloy with the desired chromium content, and to compensate for losses during the decarburization process, without, at the same time increasing the content in carbon. 40 The addition of the reduction mixture may be made in any suitable way, but it has been found preferable to add the mixture in the form of a block or similar compacted mass, so that the reaction takes place under 45 the surface of the molten metal. By this means a ferro-chrome alloy of more uniform standard may be produced and advantage is taken of the heat of the molten mass, for example the molten steel employed to mix 50 with the crude ferro-chrome, to bring the charge for the converter to the necessary temperature more quickly. Further, the addition by raising and by maintaining the heat of the molten mass facilitates the production of a homogeneous alloy. 55

It is to be understood that the invention is not restricted to crude ferro-chromes produced by any one method. For example, instead of using an electric furnace for the 60 preparation of the crude ferro-chrome, a ferro-chrome alloy which has been prepared in the blast furnace may be employed. This is not so rich in chromium, the percentage

of this metal not usually exceeding 40 per cent. Such an alloy, may, however, be treated in the converter as described, any desired augmentation of the chromium content being brought about subsequently by treatment with the thermo-reducing agent containing a chromium compound. 65 70

What I claim as my invention and desire to secure by Letters Patent is:—

1. The herein described process for the manufacture of the ferro-chrome alloy of low carbon content, which comprises submitting a molten ferro-chrome alloy of high carbon content to the action of an oxidizing blast. 75

2. The herein described process for the manufacture of a ferro-chrome alloy of low carbon content, which comprises melting a ferro-chrome alloy of higher carbon content, running the molten alloy into a converter, and submitting the molten alloy to the action of an oxidizing blast. 80

3. The herein described process for the manufacture of a ferro-chrome alloy of low carbon content, which comprises melting a ferro-chrome alloy of higher carbon content with mild basic steel, running the molten mass into a converter, and submitting the molten material to the action of an oxidizing blast. 85

4. The herein described process for the manufacture of a ferro-chrome alloy of low carbon content, which comprises submitting a molten ferro-chrome alloy of higher carbon content to the action of an oxidizing blast, and adjusting the proportion of chromium in the decarbonized alloy by treatment 100 of the latter while molten with a thermo-reduction mixture containing chromium oxid. 95

5. The herein described process for the manufacture of ferro-chrome alloy of low carbon content, which comprises melting a ferro-chrome alloy of higher carbon content with mild basic steel, running the molten mass into a converter, submitting the molten material to the action of an oxidizing blast, and adjusting the proportion of chromium in the decarbonized alloy by treatment 110 of the latter in the converter with a thermo-reduction mixture containing chromium oxid. 105

6. A process for the economical production of ferro-chrome of low carbon content, which consists in preparing ferro-chrome of high carbon content by a reduction of chromium bearing ore, running the molten alloy into a Bessemer or like converter, and subjecting it to an oxidizing blast or blowing operation to decarburize the alloy to the extent desired. 115 120

In testimony whereof I affix my signature.

WILLIAM DOWTMAN BALLANTINE.